

[54] MIDDLE DISTILLATE FUEL OIL  
COMPOSITIONS HAVING IMPROVED  
PUMPABILITY

[75] Inventor: Rodney L. Mieville, Evanston, Ill.

[73] Assignee: Standard Oil Company, Chicago, Ill.

[22] Filed: Jan. 18, 1971

[21] Appl. No.: 107,508

**Related U.S. Application Data**

[63] Continuation-in-part of Ser. No. 770,079, Oct. 23, 1968, abandoned.

[52] U.S. Cl..... 44/62, 44/70, 44/80

[51] Int. Cl..... C10I 1/18

[58] Field of Search..... 44/62, 80, 70

[56] **References Cited**

UNITED STATES PATENTS

2,049,062 7/1936 Howard ..... 44/62

|           |        |                    |       |
|-----------|--------|--------------------|-------|
| 2,379,728 | 7/1945 | Lieber et al. .... | 44/62 |
| 3,447,915 | 6/1969 | Otto.....          | 44/62 |
| 3,467,597 | 9/1969 | Tunkel et al. .... | 44/62 |
| 3,502,451 | 3/1970 | Moore et al. ....  | 44/58 |

*Primary Examiner*—Daniel E. Wyman

*Assistant Examiner*—Mrs. Y. H. Smith

*Attorney, Agent, or Firm*—Philip Hill; Arthur G. Gilkes; William T. McClain

[57]

**ABSTRACT**

Fuel oil compositions, containing a pour depressant to provide a pour point below 0°F., exhibit improved pumpability as a result of the inclusion of a minor amount of certain low molecular weight butene polymers.

4 Claims, No Drawings

**MIDDLE DISTILLATE FUEL OIL COMPOSITIONS  
HAVING IMPROVED PUMPABILITY**  
**CROSS-REFERENCE TO RELATED  
APPLICATIONS**

This application is a continuation-in-part of copending application Ser. No. 770,079 filed Oct. 23, 1968 now abandoned.

**BACKGROUND OF THE INVENTION**

In the storage and use of heavy and middle distillate fuel oils, problems connected with pour points are familiar to the art. The pour point of an oil is defined as the lowest temperature at which the oil will pour or flow when chilled without disturbance under specified conditions. Pour point problems arise through the formation of solid or semi-solid waxy particles within an oil composition. For example, in the storage of fuel oils (e.g., heater oil and furnace oil) or diesel oil during the winter months, temperatures frequently are in the range of  $-15^{\circ}$  to  $-25^{\circ}$ F. These low temperatures often cause crystallization or solidification of wax in the distillate oil.

One solution to the problem of handling oils below their natural pour point is to incorporate in the oil composition one of a wide number of known pour point depressants. In this manner it is possible to maintain flowability in a fuel even at very cold temperatures. It has been discovered, however, that pour point depressants alone are often not sufficient to permit effective handling of fuel oils at cold temperatures. This is because all hydrocarbon fuels yield crystals of solid wax as their temperature is lowered beyond the cloud point, which is defined as the temperature at which paraffin wax or other solid substances begin to crystallize out or separate from solution when the oil is chilled under definite conditions (ASTM : D 97). In many cases, even in the presence of a pour point depressant, the crystals which form are sufficiently dense so that an immobile layer of crystals is formed in the bottom of storage tanks and tends severly to clog pumps, filters and screens. Unfortunately, most pour point depressants tailored for middle distillate fuels are not effective in inhibiting such crystal growth or in modifying it in such a way as to maintain pumping capacity in the oil.

It has additionally been discovered that pumpability problems in some fuels are especially severe around the cloud point. Thus a fuel may exhibit workable pumpability at very low temperatures while being virtually non-pumpable in the warmer cloud point range.

**SUMMARY OF THE INVENTION**

This invention relates to fuel oil compositions having improved pumpability characteristics. More particularly, this invention relates to improving the pumpability of fuel oils which have already been modified to exhibit depressed pour points.

I have now discovered that certain relatively low molecular weight polybutenes, when incorporated in pour-depressed middle distillate fuel compositions at a concentration ranging from 0.005 to 0.05 weight percent, are effective in maintaining pumpability in the fuels at low temperatures and are especially effective in maintaining pumpability at or near the cloud point of the fuel.

The polybutenes of this invention are viscous liquids obtained by polymerization of  $C_4$  olefins, singly or in

combination, in the presence of a Friedel-Crafts catalyst system. The liquid polymers have a number average molecular weight within the range from about 300 to about 3,000.

**DESCRIPTION OF THE INVENTION**

The middle distillate oils with which my invention is concerned may generally be described as distillates boiling in the range from  $350^{\circ}$  to  $750^{\circ}$ F. and already 10 modified to exhibit depressed pour points below  $0^{\circ}$ F. These distillates may comprise virgin oils or cracked stocks derived, for example, from cycle oils boiling higher than gasoline. Examples of distillates suitable for use in this invention include diesel fuel (ASTM : 15 D975), jet fuel, fuel oils (ASTM : D 396), gas oils and the like. Of course, suitable distillates may additionally contain additives such as rust inhibitors, corrosion inhibitors, anti-oxidants and similar agents designed to 20 impart a specific property to the oil.

Pour point depressants suitable for modifying the middle distillates with which this invention is concerned, include any effective pour depressant known to the art. For example, such depressants may be 25 ethylene/propylene, ethylene/vinyl acetate, ethylene/aminoalkyl ester, and ethylene/acrylic acid ester copolymers. A particularly effective pour depressant is an ethylene/acrylic ester/propylene terpolymer.

The low molecular weight polybutenes which I have 30 discovered impart excellent pumpability to pour-depressed middle distillate fuel compositions, especially at or near the cloud point, have an average molecular weight in the range from about 300 to about 3,000. These polybutenes are viscous liquids generally 35 prepared by the polymerization of 1-butene, 2-butene and isobutene, either singly or in combination, in the presence of  $AlCl_3$  as catalyst.

To achieve satisfactory pumpability in difficultly-pumpable fuel compositions as described above I have 40 found it necessary to employ a minimum of about 0.005 weight percent of the described polybutene additives. In general, the polybutenes may be employed in amounts ranging from 0.005 to 0.05 weight percent, with 0.01 weight percent being a preferred amount.

I have further discovered that when a polybutene additive having a number average molecular weight of 45 about 900 is employed together with an ethylene/acrylic ester/propylene terpolymer pour point depressant in a weight ratio of about 1:10, a synergism exists which 50 results in a dramatic increase in the pumpability of the fuel composition.

**EMBODIMENTS OF THE INVENTION**

To illustrate the effectiveness of the inclusion of the 55 described polybutenes in middle distillate fuel compositions, pumpability tests were run on No. 2 fuel oils containing pour point depressants. The pumpability test employed is designed to simulate actual fuel handling conditions and is described as follows:

A tape wrapped 500 ml. leveling bulb is fitted in the 60 top with a 3-way stopcock which is wired on. The bottom of the bulb is connected by a short strip of rubber tubing to the bottom of a J-shaped piece of  $3/16$  inch copper tubing 14 inches long. The top of the copper tubing is fitted with a brass union containing a 30-mesh screen soldered into a brass washer having a  $15/32$  inch opening. The level of

the screen is at about the same height as the stopcock on the leveling bulb. A 250 ml. buret is connected to the brass union by rubber tubing.

To perform a test with this equipment, a 300 ml. fuel sample is poured into the leveling bulb and, with the stopcock open, is subjected to one of the cooling sequences shown in Table I. When cooling is complete, a nitrogen pressure of 15 p.s.i.g. is introduced through the stopcock. A pumpability reading is obtained by measuring the delivery time in seconds between the 0 and 200 ml. marks on the measuring buret.

TABLE I

| Time, Hours | GENERAL TEMPERATURE SEQUENCE |         |         |         |
|-------------|------------------------------|---------|---------|---------|
|             | T = 0                        | T = -10 | T = -20 | T = -30 |
| 0           | 75                           |         |         |         |
| 2           | 40                           |         |         |         |
| 8           | 0                            | -10     | -20     | -30     |
| 12          | 15                           |         |         |         |
| 16          | 0                            | -10     | -20     | -30     |

T = Specification Temperature

## EXAMPLE I

The pumpability of a No. 2 fuel oil having the following specifications,

|               |      |     |
|---------------|------|-----|
| Pour point,   | °F.  | -20 |
| Gravity,      | °API | 32  |
| Distillation, | °F.  |     |
| 10%           |      | 406 |
| 90%           |      | 590 |
| 95%           |      | 608 |
| EP            |      | 633 |

was determined by the procedure described above for -20°F specification temperature. The fuel had been modified to exhibit a depressed pour point of -20°F by the inclusion of 0.04 weight percent of an ethylene/a-

|            | Composition                             | Pumpability (-20°F.) |
|------------|-----------------------------------------|----------------------|
| No. 2 fuel | +0.04% pour depressant                  | Plugged, no flow     |
| No. 2 fuel | +0.04% pour depressant<br>+0.01% H-300  | 200 ml./6 seconds    |
| No. 2 fuel | +0.04% pour depressant<br>+0.01% H-1500 | 200 ml./6 seconds    |

## EXAMPLE II

10 The pumpability of three No. 2 fuel oil compositions, modified with terpolymer to exhibit depressed pour points, was determined at -5°F. and 12°F. to demonstrate the special pumpability problems often observable near the cloud point of an oil. Fuel A had the following specifications:

|              |      |      |
|--------------|------|------|
| Pour point,  | °F.  | -30  |
| Cloud point, | °F.  | 0    |
| Gravity,     | °API | 34.8 |

20 Fuel B had the following specifications:

|              |      |      |
|--------------|------|------|
| Pour point   | °F.  | -35  |
| Cloud point, | °F.  | +2   |
| Gravity,     | °API | 33.8 |

Fuel C had the following specifications:

|              |      |      |
|--------------|------|------|
| Pour point,  | °F.  | -25  |
| Cloud point, | °F.  | 0    |
| Gravity,     | °API | 34.0 |

25 All three fuels were modified to depress the pour point by the addition of 0.04 wt. percent of an ethylene/acrylic ester/propylene terpolymer. Pumpability was also determined at -5°F. after adding additionally 0.01 weight percent polybutene.

30 It appears clearly from the following table that although none of the three oils was pumpable at -5°F in the absence of the polybutene additive, all three oils were pumpable at that temperature when 0.01 weight percent of a polybutene having an average molecular weight of about 900 was included in the formulation.

| Fuel Sample                | Pumpability Test at -5°F. | Pumpability Test at 12°F. | Pumpability at -5°F. with 0.01 wt. % polybutene (MW = 900) |
|----------------------------|---------------------------|---------------------------|------------------------------------------------------------|
| Fuel A (cloud point 0°F.)  | 0 ml./60 sec.             | 200 ml./24 sec.           | 200 ml./9 sec.                                             |
| Fuel B (cloud point +2°F.) | 0 ml./60 sec.             | 200 ml./14 sec.           | 200 ml./5 sec.                                             |
| Fuel C (cloud point °F.)   | 0 ml./60 sec.             | 200 ml./15 sec.           | 200 ml./8 sec.                                             |

40 acrylic ester/propylene terpolymer. Pumpability at -20°F. was also determined after adding additionally 0.01 weight percent polybutene. Two different polybutenes were employed; H-300, having an average molecular weight of about 900, and H-1500, having an average molecular weight of about 1,200. It is clear from the data in the table below that the polybutene additives were responsible for the pumpability of the tested fuel because the fuel oil, containing only the conventional pour depressant terpolymer, did not flow at all.

60 To illustrate the synergistic effect between the polybutene additives of this invention and an ethylene/acrylic ester/propylene terpolymer, used as a pour point depressant, pumpabilities were determined at -30°F. in No. 2 fuel oil compositions containing each additive singly and in combination. The results below show a striking increase in pumpability when the polybutene was employed together with the terpolymer pour depressant.

| Fuel Composition                                                                | Pumpability at -30°F. |
|---------------------------------------------------------------------------------|-----------------------|
| Fuel + 0.10 wt. terpolymer pour depressant                                      | 0 ml./60 sec.         |
| Fuel + 0.01 wt. % polybutene (MW = 900)                                         | 0 ml./60 sec.         |
| Fuel + 0.10 wt. % terpolymer pour depressant + 0.01 wt. % polybutene (MW = 900) | 200 ml./9 sec.        |

I claim:

1. A distillate fuel composition, having improved pumpability performance at temperatures below 0°F, comprising: (a) a middle distillate fuel oil having a pour point below 0°F, said pour point having been decreased below 0°F by the addition to the fuel oil of a sufficient amount of an ethylene-acrylic ester-propylene terpolymer effective therefor, and (b) from about 0.005 to about 0.05 weight percent of a polybutene, said polybutene having a number average molecular weight within the range from about 300 to about 3,000.

10 2. The composition of claim 1 wherein the amount of polybutene in the middle distillate fuel oil is about 0.01 weight percent.

3. The composition of claim 1 wherein the number average molecular weight of the polybutene is within the range from about 900 to about 1,200.

15 4. The composition of claim 1 wherein the polybutene has a number average molecular weight of about 900, the weight ratio of terpolymer to polybutene being about 10:1.

\* \* \* \* \*

20

25

30

35

40

45

50

55

60

65